



US006569597B2

(12) **United States Patent**  
**Zheng**

(10) **Patent No.:** **US 6,569,597 B2**  
(45) **Date of Patent:** **May 27, 2003**

(54) **THERMAL IMAGING COMPOSITION AND MEMBER AND METHODS OF IMAGING AND PRINTING**

(75) Inventor: **Shiying Zheng**, Rochester, NY (US)

(73) Assignee: **Eastman Kodak Company**, Rochester, NY (US)

(\*) Notice: Subject to any disclaimer, the term of this patent is extended or adjusted under 35 U.S.C. 154(b) by 198 days.

(21) Appl. No.: **09/766,076**

(22) Filed: **Jan. 19, 2001**

(65) **Prior Publication Data**

US 2002/0142245 A1 Oct. 3, 2002

(51) **Int. Cl.<sup>7</sup>** ..... **G03F 7/038**

(52) **U.S. Cl.** ..... **430/270.1**; 430/302; 430/303; 430/348; 430/495.1; 430/944; 430/945; 430/964

(58) **Field of Search** ..... 430/270.1, 302, 430/303, 348, 495.1, 944, 945, 964; 101/130, 453, 463.1, 465, 466, 467

(56) **References Cited**

U.S. PATENT DOCUMENTS

- |              |           |                        |            |
|--------------|-----------|------------------------|------------|
| 3,636,052 A  | 1/1972    | Hatch et al. ....      | 260/323.3  |
| 3,660,431 A  | 5/1972    | Hatch et al. ....      | 260/332.3  |
| 3,813,363 A  | 5/1974    | Schmidt et al. ....    | 260/29.3   |
| 3,836,385 A  | 9/1974    | Schmidt et al. ....    | 117/47     |
| 4,118,297 A  | 10/1978   | Broxterman et al. .... | 204/159.11 |
| 4,477,640 A  | 10/1984   | Schmidt et al. ....    | 526/256    |
| 4,528,384 A  | 7/1985    | Schmidt et al. ....    | 549/78     |
| 5,985,514 A  | * 11/1999 | Zheng et al. ....      | 430/270.1  |
| 6,096,471 A  | * 8/2000  | Van Damme et al. ....  | 430/188    |
| 6,136,503 A  | * 10/2000 | Zheng et al. ....      | 430/270.1  |
| 6,159,657 A  | * 12/2000 | Fleming et al. ....    | 430/270.1  |
| 6,162,578 A  | * 12/2000 | Zheng et al. ....      | 430/270.1  |
| 6,165,679 A  | * 12/2000 | Van Damme et al. ....  | 430/270.1  |
| 6,165,691 A  | * 12/2000 | Damme et al. ....      | 430/303    |
| 6,190,830 B1 | * 2/2001  | Leon et al. ....       | 430/270.1  |
| 6,190,831 B1 | * 2/2001  | Leon et al. ....       | 430/270.1  |
| 6,399,268 B1 | * 6/2002  | Fleming et al. ....    | 430/270.1  |

6,410,202 B1 \* 6/2002 Fleming et al. .... 430/270.1  
6,423,469 B1 \* 7/2002 DoMinh et al. .... 430/270.1  
6,447,978 B1 \* 9/2002 Leon et al. .... 430/270.1  
6,451,500 B1 \* 9/2002 Leon .... 430/270.1  
2002/0068241 A1 \* 6/2002 Oohashi et al. .... 430/288.1  
2002/0123001 A1 \* 9/2002 Dorr et al. .... 430/162

FOREIGN PATENT DOCUMENTS

EP 652483 5/1995 ..... G03F/7/004  
EP 1 225 041 A2 \* 7/2002 ..... B41C/1/10

\* cited by examiner

*Primary Examiner*—Janet Baxter

*Assistant Examiner*—Barbara Gilliam

(74) *Attorney, Agent, or Firm*—J. Lanny Tucker

(57) **ABSTRACT**

An imaging member, such as a negative-working printing plate or on-press cylinder, has an imaging layer comprised of a thermally sensitive compound and a photothermal conversion material. The thermally sensitive compound comprises a heat-activatable aromatic cyclic sulfonium zwitterion group represented by the following Structure I:



wherein Ar is a substituted or unsubstituted aromatic group, X and Y are independently substituted or unsubstituted methylene groups, and n is 1 or 2. The thermally sensitive compound can be a polymer or a small molecule compound. In the imaging member, the thermally sensitive compound reacts to provide increased hydrophobicity in areas exposed to energy that provides or generates heat. The imaging layer is considered “switchable” and can be used to provide a lithographic printing image without traditional alkaline wet processing.

**29 Claims, No Drawings**

**THERMAL IMAGING COMPOSITION AND MEMBER AND METHODS OF IMAGING AND PRINTING**

**FIELD OF THE INVENTION**

This invention relates in general to thermal imaging compositions, and to direct-write imaging members (particularly lithographic printing plates) prepared therefrom. The invention also relates to a method of imaging such imaging members, and to a method of printing using them, with or without processing after imaging.

**BACKGROUND OF THE INVENTION**

The art of lithographic printing is based upon the immiscibility of oil and water, wherein an oily material or ink is preferentially retained by an imaged area and the water or fountain solution is preferentially retained by the non-imaged areas. When a suitably prepared surface is moistened with water and ink is applied, the background or non-imaged areas retain the water and repel the ink while the imaged areas accept the ink and repel the water. The ink is then transferred to the surface of a suitable substrate, such as cloth, paper or metal, thereby reproducing the image.

Very common lithographic printing plates include a metal or polymer support having thereon an imaging layer sensitive to visible or UV light. Both positive- and negative-working printing plates can be prepared in this fashion. Upon exposure to a patterned light image, and perhaps post-exposure heating, either imaged or non-imaged areas are removed using wet processing chemistries.

“Direct-write” imaging avoids the need for patterned light imaging and chemical processing. Direct-write using an infrared radiation laser is a thermally driven process and is more desirable because the laser heats only a small region at a time. Moreover, computer control allows for high resolution images to be generated at high speed since the images can be produced directly on the imaging member surface, pixel by pixel. The chemical processing steps are eliminated.

Examples of thermally sensitive printing plates are described in U.S. Pat. No. 5,372,915 (Haley et al.). They include an imaging layer comprising a mixture of dissolvable polymers and an infrared radiation absorbing compound. While these plates can be imaged using lasers and digital information, they still require wet processing using alkaline developer solutions.

It has been recognized that a lithographic printing plate could be created by ablating an IR absorbing layer. For example, Canadian 1,050,805 (Eames) discloses a dry planographic printing plate comprising an ink receptive substrate, an overlying silicone rubber layer, and an interposed layer comprised of laser energy absorbing particles (such as carbon particles) in a self-oxidizing binder (such as nitrocellulose). Such plates were exposed to focused near IR radiation with a Nd<sup>3+</sup>-YAG laser. The absorbing layer converted the infrared energy to heat thus partially loosening, vaporizing or ablating the absorber layer and the overlying silicone rubber. Similar plates are described in *Research Disclosure* 19201, 1980 as having vacuum-evaporated metal layers to absorb laser radiation in order to facilitate the removal of a silicone rubber overcoated layer. These plates were developed by wetting with hexane and rubbing. Other publications describing ablative printing plates include U.S. Pat. No. 5,385,092 (Lewis et al.), U.S. Pat. No. 5,339,737 (Lewis et al.), U.S. Pat. No. 5,353,705 (Lewis et al.), U.S. Reissue No. 35,512 (Nowak et al.), and U.S. Pat. No. 5,378,580 (Leenders).

While the noted printing plates used for digital, processless printing have a number of advantages over the more conventional photosensitive printing plates, there are a number of disadvantages with their use. The process of ablation creates debris and vaporized materials that must be collected. The laser power required for ablation can be considerably high, and the components of such printing plates may be expensive, difficult to coat, or unacceptable for resulting printing quality. Such plates generally require at least two coated layers on a support.

U.S. Pat. No. 3,650,743 (Hallman et al.) and U.S. Pat. No. 4,115,127 (Ikeda et al.) describe printing plates that do not require post-imaging processing. However, these imaging members are constructed of toxic materials such as arsenic that must be applied by vacuum deposition of mixed inorganic coating formulations.

Thermal or laser mass transfer is another method of preparing processless lithographic printing plates. Such methods are described for example in U.S. Pat. No. 5,460,918 (Ali et al.) wherein a hydrophobic image is transferred from a donor sheet to a microporous hydrophilic crosslinked silicated surface of the receiver sheet. U.S. Pat. No. 3,964,389 (Peterson) describes a process of laser transfer of an image from a donor material to a receiver material requiring a high temperature post-heating step.

Still another method of imaging that avoids chemical processing is the use of materials comprising microencapsulated hydrophobic materials as described for example in U.S. Pat. No. 5,569,573 (Takahashi et al.). Upon thermal imaging, the microcapsules rupture in an imagewise fashion to provide an ink-receptive image.

Thermally switchable polymers have been described for use as imaging materials in printing plates. By “switchable” is meant that the polymer is rendered from hydrophobic to relatively more hydrophilic or, conversely from hydrophilic to relatively more hydrophobic, upon exposure to heat. U.S. Pat. No. 4,034,183 (Uhlig) describes the use of high powered lasers to convert hydrophilic surface layers to hydrophobic surfaces. A similar process is described for converting polyamic acids into polyimides through a transparency mask in U.S. Pat. No. 4,081,572 (Pacansky). The use of high-powered lasers is undesirable in the industry because of their high electrical power requirements and because of their need for cooling and frequent maintenance.

U.S. Pat. No. 4,634,659 (Esumi et al.) describes imagewise irradiating hydrophobic polymer coatings to render exposed regions more hydrophilic in nature. While this concept was one of the early applications of converting surface characteristics in printing plates, it has the disadvantages of requiring long UV light exposure times (up to 60 minutes), and the plate’s use is in a positive-working mode only.

U.S. Pat. No. 4,405,705 (Etoh et al.) and U.S. Pat. No. 4,548,893 (Lee et al.) describe amine-containing polymers for photosensitive materials used in non-thermal processes. Thermal processes using polyamic acids and vinyl polymers with pendant quaternary ammonium groups are described in U.S. Pat. No. 4,693,958 (Schwartz et al.). Such materials require aqueous processing after imaging. U.S. Pat. No. 5,512,418 (Ma) describes the use of polymers having cationic quaternary ammonium groups that are heat-sensitive. However, the materials described in this art require wet processing after imaging.

WO 92/09934 (Vogel et al.) describes photosensitive compositions containing a photoacid generator and a polymer with acid labile tetrahydropyranyl or activated ester

groups. However, imaging of these compositions converts the imaged areas from hydrophobic to hydrophilic in nature.

EP-A 0 652 483 (Ellis et al.) describes direct-write lithographic printing plates imageable using IR lasers, and that do not require wet processing. These plates comprise an imaging layer that becomes more hydrophilic upon image-wise exposure to heat. This coating contains a polymer having pendant groups (such as t-alkyl carboxylates) that are capable of reacting under heat or acid to form more polar, hydrophilic groups. Imaging such compositions converts the imaged areas from hydrophobic to relatively more hydrophilic in nature, and thus requires imaging the background of the plate, which is generally a larger area. This can be a problem when imaging to the edge of the printing plate is desired. Moreover, the polymers described by Ellis et al. suffer from short shelf life and are difficult to manufacture.

The graphic arts industry is seeking an alternative means for providing processless, direct-write, negative-working lithographic imaging members that can be imaged without ablation, or the other problems noted above, to provide high sensitivity, high imaging speed, long shelf life, and long press life.

#### SUMMARY OF THE INVENTION

The problems noted above are overcome with a heat-sensitive composition comprising:

- a) a thermally sensitive compound comprising a heat-activatable aromatic cyclic sulfonium zwitterion group represented by the following Structure I:



wherein Ar is a substituted or unsubstituted aromatic group, X and Y are independently substituted or unsubstituted methylene groups, and n is 1 or 2, and

- b) a photothermal conversion material.

This invention also provides a thermally sensitive imaging member comprising a support having disposed thereon an imaging layer comprising the thermally sensitive compound of Structure I described above, and a photothermal conversion material in the same or different layer.

This invention further provides a thermally sensitive imaging member comprising a support and having disposed thereon a heat-sensitive imaging layer that is prepared from the heat-sensitive composition described above.

Still further, this invention includes a method of imaging comprising the steps of:

- A) providing an imaging member as described above, and B) image-wise exposing the imaging member to thermal energy to provide exposed and unexposed areas in the imaging layer of the imaging member, whereby the exposed areas are rendered more hydrophobic than the unexposed areas.

A method of printing comprises the steps of carrying out steps A and B noted above, and additionally:

- C) with or without wet processing, contacting the image-wise exposed imaging member with a lithographic printing ink, and image-wise transferring that printing ink from the imaging member to a receiving material.

The negative-working imaging members of this invention have a number of advantages and avoid the problems of previous printing plates. Specifically, the problems and concerns associated with ablation imaging (that is, image-wise removal of a surface layer) are avoided because imaging is accomplished in the imaging layer by "switching" (preferably, irreversibly) exposed relatively hydrophilic areas of the printing surface to a more hydrophobic (more ink-receptive) nature upon heating. Thus, the imaging layer stays intact during and after imaging (that is, no ablation occurs).

The thermally sensitive compounds having a heat-activatable group represented by Structure I used in the practice of this invention (both polymers and small molecule compounds) can be readily prepared or purchased from a number of commercial sources. Thus, the imaging members are simple to make and can be used with or without post-imaging wet processing. The resulting printing members formed from the imaging members of this invention are generally negative working in nature. Moreover, the imaging members are durable because upon heating, the heat-sensitive compounds described above not only provide hydrophobicity, but they react with each other, or crosslink, in the exposed areas.

#### DETAILED DESCRIPTION OF THE INVENTION

##### Definitions:

"Photothermal conversion materials" are inorganic or organic compounds that absorb radiation from an appropriate energy source (such as a laser) and converts that radiation into heat. More details of such compounds are provided below.

As known in the lithographic printing art, materials that release or repel oil-based inks are referred to as having "oleophobic", "hydrophilic", or "ink-repelling" character, and conversely, materials that accept oil-based inks are referred to as "oleophilic" or "hydrophobic."

"Wet processing" refers to washing off unexposed regions of the imaging layer after imaging using water or a fountain solution. It does not refer to contacting the imaging member with alkaline developers or other chemical processing solutions used in conventional lithographic developing methods.

The imaging members of this invention comprise a support and one or more layers thereon that include a dried thermally sensitive composition as described herein. The support can be any self-supporting material including polymeric films, glass, ceramics, cellulosic materials (including papers), metals or stiff papers, or a lamination of any of these materials. The thickness of the support can be varied and should be sufficient to sustain the wear from printing and thin enough to wrap around a printing form. A preferred embodiment uses a polyester support prepared from, for example, polyethylene terephthalate or polyethylene naphthalate, and having a thickness of from about 100 to about 310  $\mu\text{m}$ . Another preferred embodiment uses aluminum sheets having a thickness of from about 100 to about 600  $\mu\text{m}$ . The support should resist dimensional change under conditions of use. The aluminum and polyester supports are most preferred for the imaging members of this invention.

The support may also be a cylindrical support that includes printing cylinders on press as well as printing sleeves that are fitted over printing cylinders. The use of such supports to provide cylindrical imaging members is described in U.S. Pat. No. 5,713,287 (Gelbart). The thermally sensitive composition of this invention can be coated or sprayed directly onto the cylindrical surface that is an integral part of the printing press.

The support may be coated with one or more "subbing" layers to improve adhesion of the final assemblage. Examples of subbing layer materials include, but are not limited to, gelatin and other naturally occurring and synthetic hydrophilic colloids and vinyl polymers (such as vinylidene chloride copolymers) that are known for such purposes in the photographic industry, vinylphosphonic acid polymers, sol gel materials such as those prepared from alkoxy silanes (including glycidoxypropyltriethoxysilane and aminopropyltriethoxysilane), epoxy functional polymers, and various ceramics. The support can also have thereon conventional reflecting layers such as layers of evaporated metals, or an IR radiation reflection layer.

The backside of the support may be coated with antistatic agents and/or slipping layers or matte layers to improve handling and "feel" of the imaging member.

The imaging members, however, preferably have only one layer on the support, that is a heat-sensitive surface layer that is required for imaging. This layer is prepared from a heat-sensitive composition of this invention and includes one or more thermally sensitive compounds and one or more photothermal conversion materials (both described below) as the only essential components for imaging. Because of the particular thermally sensitive compounds used in the imaging layer, the exposed (imaged) areas of the layer are rendered more hydrophobic in nature. The unexposed areas remain relatively hydrophilic in nature and can be washed off using water or a fountain solution if desired.

In an alternative embodiment, the imaging member comprises one or more thermally sensitive compounds as described herein in a surface imaging layer, and one or more photothermal conversion materials in a separate layer directly underneath, or in thermal contact with, the imaging layer. The photothermal conversion materials can diffuse into the imaging layer prior to or during imaging.

The thermally sensitive compounds useful in the imaging members of this invention can be one or more polymers or one or more small molecular compounds (non-polymeric), or the blend of both types of compounds. Useful heat-sensitive polymers can be vinyl homopolymers or copolymers prepared from one or more ethylenically unsaturated polymerizable monomers that are reacted together using known polymerization techniques. Alternatively, they can be addition homopolymers or copolymers prepared from one or more heterocyclic monomers that are reacted together using known polymerization techniques (such as polyethers or polythioethers). Additionally, they can be condensation type polymers (such as polyesters, polythioester, polyimides, polyamides, polyurethanes, polyketones, polycarbonates, polyanhydrides, polysulfones, polysulfines, polyureas, or phenol-formaldehyde resin) prepared using known polymerization procedures and conditions.

Whether the compounds are small molecular compounds or polymers, they comprise one or more heat-activatable aromatic cyclic zwitterion groups as represented by the following Structure I:



5

10

15

20

25

30

35

40

45

50

55

60

65

wherein Ar is a substituted or unsubstituted aromatic carbocyclic or heterocyclic group that generally has from 6 to 18 carbon atoms in the aromatic ring system (such as phenyl, naphthyl, anthryl, phenanthryl, pyrenyl, crysenyl, triphenyl, benzanthryl, and biphenyl). Preferably, Ar is a substituted or unsubstituted phenyl or naphthyl group. Depending upon the type of thermally sensitive compound being used, Ar can represent either a monovalent or divalent aromatic group (for example, aryl" or "arylene" group). The various substituents on Ar can be any of those defined below for the "R" group for Structure II.

Structure I also represents dimer compounds in which two of the illustrated moieties are directly linked through the Ar groups, or by means of a linking group like Z defined below.

If the thermally sensitive compound is a thermally sensitive polymeric material, it can be represented by the following Structure II:



wherein A represents a polymeric backbone from any of the type of polymers described above. Preferably, A represents a vinyl polymer binder.

In Structure II, Ar' represents a divalent aromatic group that is defined similar to Ar. R represents the same or different substituent on said aromatic group. Representative useful R groups are defined below. Moreover, m is 0 or an integer representing available open ring positions on Ar'. Preferably, m is 0 or 1 to 3, and more preferably, m is 0, 1 or 2.

The heat-activatable aromatic cyclic sulfonium zwitterion group can be directly attached to the polymeric backbone (that is, q is 0), or it can be attached by means of the divalent linking group "Z" (that is, q is 1). Preferably, q is 1.

Z is  $-(Z)_p Z'$ , wherein Z' is an oxy ( $-O-$ ), thio ( $-S-$ ), carboxyloxy ( $-COO-$ ), oxycarbonyl ( $-OCO-$ ), carbonyl ( $-CO-$ ), carboxyloxy carbonyl ( $-COOCO-$ ),  $-SO-$ ,  $-SO_2-$ ,  $-NHCONH-$ , or carbonamido ( $-CONH-$ ) group. Preferably, Z' is a carboxyloxy group. The hydrogen atoms on the carbonamido and  $-NHCONH-$  groups can be replaced with any of the groups described above for R.

Z' is a substituted or unsubstituted alkylene, substituted or unsubstituted arylene, substituted or unsubstituted arylenealkylene, or substituted or unsubstituted alkylene-arylene group, each group having up to 20 carbon atoms in the chain linking the polymer backbone to the heat-activatable group. Thus, representative Z' groups include, but are not limited to, substituted or unsubstituted

methylene, ethylene, n-butylene, isopropylene, phenylene, naphthylene, anthracylene, xylylene, p-methylenephylene, p-phenylenemethylene, phenylenemethylenephenylene, biphenylene, phenyleneisopropylenephenylene, 1,4-dimethylenephylene, and terphenylene. Preferably,  $Z''$  is a substituted or unsubstituted alkylene or arylene group, and more preferably, it is a substituted or unsubstituted alkylene group having 1 to 6 carbon atoms (including linear and branched groups), a substituted phenylene or naphthylene group, or a substituted or unsubstituted phenylenealkylene group having 7 or 8 atoms in the linking chain.

In addition,  $p$  and  $t$  are independently 0 or 1, and preferably, each is 1.

More preferred  $Z$  groups are  $—COO—$  or  $—COO—Z''$  groups wherein  $Z''$  is an alkylene group having 1 or 2 carbon atoms, a phenylene group, or a naphthylene group. Most preferably,  $Z$  is  $—COO—$ .

Ar and  $Ar'$  can be substituted with one or more monovalent substituents, the number and type of substituents are limited only by the available valences on the aromatic ring and they do not adversely affect the desired imaging properties of the thermally sensitive compounds. For example, such substituents (shown as "R" in Structure II) can be a halo (such as fluoro, chloro, or bromo) group, an alkyl group generally having 1 to 16 carbon atoms (including linear and branched monovalent alkyl groups that can be further substituted with any substituents described herein), an aryl group generally having 1 to 18 carbon atoms in the ring system (including those groups described for Ar), an alkoxy group generally having 1 to 16 carbon atoms (including linear and branched monovalent alkyl groups that can be further substituted with any of the substituents described herein), a substituted or unsubstituted alkyl or aryl ester group (such as carbonyloxymethyl, carbonyloxyphenyl, oxy carbonylethyl, and oxy carbonylphenyl), a primary, secondary or tertiary amine, a thioether group, or a thioester group.

Preferably, Ar and  $Ar'$  are substituted with 1 to 3 chloro, bromo, or substituted or unsubstituted alkyl groups having 1 to 4 carbon atoms (both linear and branched groups).

In both Structures I and II, X and Y are independently substituted or unsubstituted methylene groups (such as  $—CH_2—$  or  $—CHR—$ ), and  $n$  is 1 or 2, wherein R is as defined above. Preferably, each of X and Y is  $—CH_2—$ , and  $n$  is 1.

Representative small molecule thermally sensitive compounds useful in the present invention from Structure I can be illustrated by the following types of compounds of Structures I-a through I-k wherein R, Z, q, and m are defined above:



9

-continued



10

-continued

2

I-h

5



I-i 15

10



I-j

20



I-k

25



30

35

40

45

3

4

5

Mixtures of such compounds can be used if desired in the imaging members of this invention.

The following non-polymeric, small molecule Compounds 1-5 useful in the present invention were specifically prepared in the Synthetic Examples described below:



The heat-sensitive polymers useful in the practice of this invention include polymer recurring units that comprise the heat-activatable aromatic cyclic sulfonium zwitterion groups as illustrated in Structure II above. The polymers can include more than one type of recurring unit that comprise such groups. In addition, they can include polymer recurring units that do not comprise such groups. Generally, at least 10 mol %, preferably from about 15 to 100 mol %, and more preferably from about 20 to 100 mol %, of all recurring units in the polymers comprise the noted heat-activatable groups. The recurring units can be derived from polymerizable monomers that contain the heat-activatable groups, or they can be derived from monomers that, after polymerization, can be modified to provide the heat-activatable groups. Mixtures of such polymers can be used in the imaging members of this invention if desired.

Preferred heat-sensitive polymers are vinyl polymers derived from one or more ethylenically unsaturated polymerizable monomers and can be represented by the following Structure III:



wherein X' represents recurring units to which the heat-activatable aromatic cyclic sulfonium zwitterion groups of Structure I (represented by "SULFO" in Structure III) are attached, and Y' represents recurring units derived from any additional ethylenically unsaturated polymerizable monomers. The various repeating units are present in suitable amounts, as represented by x being from about 10 to 100 mol %, and y being from 0 to about 90 mol %. Preferably, x is from about 20 to 100 mol %, and y is from 0 to about 80 mol %.

While the heat-activatable groups in the polymers are crosslinked in imaged areas of the imaging member, additional crosslinking can be provided in a number of ways if desired as long as this crosslinking does not interfere with the transformation of the aromatic cyclic sulfonium zwitterion groups during imaging. There are numerous monomers and methods for crosslinking that are familiar to one skilled in the art. Some representative crosslinking strategies include, but are not necessarily limited to:

- a) reacting an amine or carboxylic acid or other Lewis basic units with diepoxide crosslinkers,
- b) reacting epoxide units within the polymer with difunctional amines, carboxylic acids, or other difunctional Lewis basic unit,
- c) irradiative or radical-initiated crosslinking of double bond-containing units such as acrylates, methacrylates, cinnamates, or vinyl groups,
- d) reacting a multivalent metal salts with ligating groups within the polymer (the reaction of zinc salts with carboxylic acid-containing polymers is an example),
- e) using crosslinkable monomers that react via the Knoevenagel condensation reaction, such as (2-acetoacetoxy)ethyl acrylate and methacrylate,
- f) reacting an amine, thiol, or carboxylic acid groups with a divinyl compound (such as bis (vinylsulfonyl) methane) via a Michael addition reaction,
- g) reacting a carboxylic acid units with crosslinkers having multiple aziridine units,
- h) reacting a crosslinkers having multiple isocyanate units with amines, thiols, or alcohols within the polymer,
- i) mechanisms involving the formation of interchain sol-gel linkages [such as the use of the 3-(trimethoxysilyl) propylmethacrylate monomer],
- j) oxidative crosslinking using an added radical initiator (such as a peroxide or hydroperoxide),
- k) autoxidative crosslinking, such as employed by alkyd resins,
- l) sulfur vulcanization, and
- m) processes involving ionizing radiation.

Polymerizable monomers having crosslinkable groups or active crosslinkable sites (or groups that can serve as attachment points for crosslinking additives, such as epoxides) can be copolymerized with the other monomers noted above. Such polymerizable monomers include, but are not limited to, 3-(trimethoxysilyl)propyl acrylate or methacrylate, cinnamoyl acrylate or methacrylate, N-methoxymethyl methacrylamide, N-aminopropylacrylamide hydrochloride, acrylic or methacrylic acid and hydroxyethyl methacrylate.

Other additional polymerizable monomers that can provide the recurring units represented by "Y" in the Structure

III above include any useful hydrophilic or oleophilic ethylenically unsaturated polymerizable monomer that may provide desired physical or printing properties to the hydrophilic imaging layer. Such monomers include, but are not limited to, acrylates and methacrylates (such as ethyl acrylate, ethyl methacrylate, n-butyl acrylate, methyl methacrylate, t-butyl methacrylate, and n-butyl methacrylate), acrylonitrile and methacrylonitrile, styrene and styrene derivatives, acrylamides and methacrylamides, vinyl ethers, vinyl pyridines, vinyl pyrrolidones, vinyl acetate, vinyl halides (such as vinyl chloride, vinylidene chloride, and vinyl bromide), and dienes (such as ethylene, propylene, 1,3-butadiene, and isobutylene). Acrylates, acrylamides and styrene (and its derivatives) are preferred.

Preferred general polymeric thermally sensitive compounds useful in the present invention include, but are not limited to, those represented by the following Structures II-a to II-f:



13

-continued



Mixtures of these polymers can be used in the imaging members of this invention if desired.

The following specific polymeric thermally sensitive compounds 6–8 were prepared in the Synthetic Examples below:



14

-continued

8

II-e

5



10

II-f

15

A mixture of thermally sensitive compounds can also be used in the imaging layer. Such mixtures can include one or more non-polymeric, small molecule thermally sensitive compounds, one or more thermally sensitive polymers, or one or more small molecule compounds with one or more polymeric compounds.

The thermally sensitive compounds described herein having the aromatic cyclic sulfonium zwitterion groups are believed to polymerize and switch from relatively hydrophilic to relatively hydrophobic upon exposure to thermal energy that provides or generates heating. Hence, the imaging members of this invention are negative working imaging members.

Thermally sensitive compounds comprising five-membered cyclic sulfonium groups can be prepared by the reaction of a phenolic compound with tetrahydrothiophene 1-oxide and hydrogen chloride or with tetrahydrothiophene and chloride. The resulting hydrochloride salts are converted to the zwitterions using an ion-exchange resin or by neutralization using sodium methoxide. The compounds comprising six-membered cyclic sulfonium groups can be synthesized from the reaction of 1,5-dibromopentanes with methylthiophenolic compounds in refluxing chlorobenzene. The general synthetic procedures are described in U.S. Pat. No. 3,636,052 (Hatch), incorporated herein by reference. Polymers containing the heat-activatable aromatic cyclic sulfonium zwitterions can be prepared either from functional monomers or from preformed polymers as described above.

Representative synthetic methods for thermally sensitive polymers and small molecule compounds containing active aromatic cyclic sulfonium zwitterions useful in the practice of this invention are illustrated below just before the Examples.

The imaging layer of the imaging member can also include minor amounts (less than 20 weight %, based on total dry weight of the layer) of additional binder or polymeric materials that will not adversely affect its imaging or printing characteristics. However, the imaging layer comprises no additional materials that are needed for imaging, especially those materials (such as novolak or resole resins) commonly used for wet processing with alkaline developer solutions.

In the thermally sensitive composition (including solvent) used to provide the heat-sensitive layer, the amount of thermally sensitive compound is generally present in an amount of at least 1% solids, and preferably at least 2% solids. A practical upper limit of the amount of charged polymer in the composition is 90% solids.

The amount of thermally sensitive compound(s) present in the dried imaging layer is generally at least 0.1 g/m<sup>2</sup>, and

## 15

preferably from about 0.1 to about 10 g/m<sup>2</sup> (dry weight). The dried imaging layer generally has an average dry thickness of from about 0.1 to about 10 m. Greater amounts can be used if desired.

The imaging and any other layers in the imaging member can also include one or more conventional surfactants for coatability or other properties, dyes or colorants to allow visualization of the written image, or any other addenda commonly used in the lithographic art, as long as the concentrations are low enough so they are inert with respect to imaging or printing properties.

It is essential that the imaging member include one or more photothermal conversion materials. Preferably, they absorb radiation in the infrared and near-infrared regions of the electromagnetic spectrum. The photothermal conversion materials useful in this invention include infrared radiation (IR) dyes, carbon black, polymer grafted carbon, pigments, evaporated pigments, semiconductor materials, alloys, metals, metal oxides, metal sulfides or combinations thereof, or a dichroic stack of materials that absorb radiation by virtue of their refractive index and thickness. Borides, carbides, nitrides, carbonitrides, bronze-structured oxides and oxides structurally related to the bronze family but lacking the WO<sub>29</sub> component, are also useful. Useful absorbing dyes for near infrared diode laser beams are described, for example, in U.S. Pat. No. 4,973,572 (DeBoer). Particular dyes of interest are "broad band" dyes, that is those that absorb over a wide band of the spectrum. Mixtures of one or more types of these compounds can be

used if desired. Carbon blacks and IR dyes are preferred photothermal conversion materials.

Still other useful photothermal conversion materials include multisulfonated IR dyes as described U.S. Pat. No. 6,159,657 (Fleming et al.), the disclosure of which is incorporated herein by reference.

Useful IR-dyes are sensitive to radiation in the near-infrared and infrared regions of the electromagnetic spectrum. Thus, they are generally sensitive to radiation at or above 700 nm (preferably from about 800 to about 900 nm, and more preferably from about 800 to about 850 nm).

Examples of useful IR dyes of several classes include, but are not limited to, bis(dichlorobenzene-1,2-thiol)nickel(2:1) tetrabutyl ammonium chloride, tetrachlorophthalocyanine aluminum chloride, and the following compounds:

IR Dye 1



IR Dye 2 is the same as IR Dye 1 but with C<sub>3</sub>F<sub>7</sub>CO<sub>2</sub><sup>-</sup> as the anion.

IR Dye 4



IR Dye 5



IR Dye 6





IR Dye 8



IR Dye 9



IR Dye 10



IR Dye 11



-continued

IR Dye 12



IR Dye 13



IR Dye 14



40

IR Dyes 1–7 can be prepared using known procedures or obtained from several commercial sources (for example, Esprit, Sarasota, Fla.). IR dyes 8–14 can be prepared using known procedures, as described for example in U.S. Pat. No. 4,871,656 (Parton et al.) and reference noted therein (for example, U.S. Pat. No. 2,895,955, U.S. Pat. No. 3,148,187 and U.S. Pat. No. 3,423,207), all incorporated by reference.

As noted above, the one or more photothermal conversion materials can be included in a separate layer that is in thermal contact with the heat-sensitive imaging layer. Thus, during imaging, the action of the additional photothermal conversion material can be transferred to the heat-sensitive imaging layer.

Wherever the photothermal conversion materials are located, they are generally present in an amount sufficient to provide an optical density of at least 0.1, and preferably of at least 1.0. The particular amount required for a given material and formulation could be readily determined by a skilled worker in the art using routine experimentation. In the heat-sensitive formulation used to provide heat-sensitive imaging layers, the photothermal conversion material(s) is generally present in an amount of from about 5 to about 35% of the total solids (prior to drying).

The thermally sensitive composition of this invention can be applied to a support using any suitable equipment and procedure, such as spin coating, knife coating, gravure coating, dip coating or extrusion hopper coating. In addition,

the composition can be sprayed onto a support, including an on-press cylindrical support (such as an on-press cylinder or sleeve), using any suitable spraying means for example as described in U.S. Pat. No. 5,713,287 (noted above) to provide an imaging member. Exposure can occur as in Step B described above.

The thermally sensitive compositions of this invention are generally formulated in and coated from water or water-miscible organic solvents including, but not limited to, water-miscible alcohols (for example, methanol, ethanol, isopropanol, 1-methoxy-2-propanol and n-propanol), methyl ethyl ketone, tetrahydrofuran, acetonitrile and acetone. Water, methanol, ethanol and 1-methoxy-2-propanol are preferred. Mixtures (such as a mixture of water and methanol) of these solvents can also be used if desired. By "water-miscible" is meant that the organic solvent is miscible in water at all proportions at room temperature.

The imaging members of this invention can be of any useful form including, but not limited to, printing plates, printing cylinders, printing sleeves and printing tapes (including flexible printing webs), all of any suitable size or dimensions. Preferably, the imaging members are lithographic printing plates having an aluminum support or on-press cylinders.

During use, the imaging member of this invention is exposed to a suitable source of energy that generates or provides heat, such as a focused laser beam or a thermore-

sistive head (or "thermal head"), in the foreground areas where ink is desired in the printed image, typically from digital information supplied to the imaging device. A laser used to expose the imaging member of this invention is preferably a diode laser, because of the reliability and low maintenance of diode laser systems, but other lasers such as gas or solid state lasers may also be used. The combination of power, intensity and exposure time for laser imaging would be readily apparent to one skilled in the art. Specifications for lasers that emit in the near-IR region, and suitable imaging configurations and devices are described in U.S. Pat. No. 5,339,737 (Lewis et al.), incorporated herein by reference. The imaging member is typically sensitized so as to maximize responsiveness at the emitting wavelength of the laser.

The imaging apparatus can operate on its own, functioning solely as a platemaker, or it can be incorporated directly into a lithographic printing press. In the latter case, printing may commence immediately after imaging, thereby reducing press set-up time considerably. The imaging apparatus can be configured as a flatbed recorder or as a drum recorder, with the imaging member mounted to the interior or exterior cylindrical surface of the drum.

In the drum configuration, the requisite relative motion between an imaging device (such as laser beam) and the imaging member can be achieved by rotating the drum (and the imaging member mounted thereon) about its axis, and moving the imaging device parallel to the rotation axis, thereby scanning the imaging member circumferentially so the image "grows" in the axial direction. Alternatively, the beam can be moved parallel to the drum axis and, after each pass across the imaging member, increment angularly so that the image "grows" circumferentially. In both cases, after a complete scan by the laser beam, an image corresponding to the original document or picture can be applied to the surface of the imaging member.

In the flatbed configuration, a laser beam is drawn across either axis of the imaging member, and is indexed along the other axis after each pass. Obviously, the requisite relative motion can be produced by moving the imaging member rather than the laser beam.

While laser imaging is preferred in the practice of this invention, imaging can be provided by any other means that provides or generates thermal energy in an imagewise fashion. For example, imaging can be accomplished using a thermoresistive head (thermal printing head) in what is known as "thermal printing", described for example in U.S. Pat. No. 5,488,025 (Martin et al.). Such thermal printing heads are commercially available (for example, as Fujitsu Thermal Head FTP-040 MCS001 and TDK Thermal Head F415 HH7-1089).

Imaging on printing press cylinders can be accomplished using any suitable means, for example, as taught in U.S. Pat. No. 5,713,287 (noted above), that is incorporated herein by reference.

After imaging, the imaging member can be used for printing without conventional wet processing. Unexposed areas in the imaging surface can be washed away if desired using a conventional fountain solution. Applied ink can be imagewise transferred to a suitable receiving material (such as cloth, paper, metal, glass or plastic) to provide one or more desired impressions. If desired, an intermediate blanket roller can be used to transfer the ink from the imaging member to the receiving material. The imaging members can be cleaned between impressions, if desired, using conventional cleaning means.

The following synthetic examples are presented to show how some of the preferred thermally sensitive compounds can be prepared.

## SYNTHESIS EXAMPLE 1

## Synthesis of Compounds 1-5

1-Naphthol (27.7 g, 0.19 mol) was dissolved in absolute methanol (200 ml) and cooled to -10° C. in an ice-salt bath. The resulting solution was bubbled with dry HCl gas until saturation and then a catalytic amount of aluminum chloride was added. Tetrahydrothiophene 1-oxide (20.0 g, 0.19 mol) was added slowly through an additional funnel to keep the temperature below 0° C. After 2 hours, the reaction was stopped and the solvent was evaporated under reduced pressure at about 40° C. until a thick slurry of crystalline material was obtained. Acetone was then added and the desired hydrochloride salt was isolated as off-white crystals (24.0 g, 47% yield). <sup>1</sup>H NMR (CD<sub>3</sub>OD) δ ppm: 2.32-2.38 (m, 2H), 2.50-2.55 (m, 2H), 3.61-3.69 (m, 2H), 3.96-4.05 (m, 2H), 7.02 (d, J=8.4 Hz, 2H), 7.50-7.55 (m, 2H), 7.64-7.69 (m, 2H), 7.86 (d, J=8.5 Hz, 2H), 8.20 (d, J=8.5 Hz, 2H), 8.25 (d, J=8.4 Hz, 2H).

The hydrochloride salt was then dissolved in methanol (200 ml) and passed through Dowex-OH basic ion-exchange resin to increase the pH to about 10. Solvent was evaporated and acetone was added. The desired Compound 1 was collected as off-white crystals (14.0 g, 69% yield). A toxic by-product was removed according to the teaching of U.S. Pat. No. 4,968,433 (Schmidt). <sup>1</sup>H NMR (CD<sub>3</sub>OD) δ ppm: 2.06-2.14 (m, 2H), 2.31-2.38 (m, 2H), 3.16-3.24 (m, 2H), 3.60-3.68 (m, 2H), 6.50 (d, J=8.8 Hz, 2H), 7.44 (d, J=8.8 Hz, 2H), 7.83 (d, J=8.4 Hz, 2H), 8.24 (d, J=8.4 Hz, 2H).

Compounds 2-5 were similarly prepared.

## SYNTHESIS EXAMPLE 2

## Synthesis of Precursor Compound A

Catechol (20.0 g, 0.18 mol) was dissolved in dioxane (450 ml). To this solution were added sodium hydroxide (18.2 g, 0.45 mol) and tetrabutylammonium hydrogen sulfate (0.46 g, 0.001 mol, catalytic amount). To the mixture was added methacryloyl chloride (19.0 g, 0.18 mol) in 150 ml of dioxane through an additional funnel. The reaction was stirred at room temperature overnight. The precipitate from the reaction was filtered off and the filtrate was evaporated. The crude product was purified by column chromatography on silica gel using 10:90 ether:hexane mixture as an eluent to give 16.1 g of Precursor Compound A (shown below) as an off-white solid (50% yield). <sup>1</sup>H NMR (CD<sub>3</sub>OD) δ ppm: 2.04 (s, 3H), 5.75 (s, vinyl H, 1H), 6.34 (s, vinyl H, 1H), 6.53-6.63 (m, 3H), 6.93 (s, br, OH, 1H), 7.11-7.16 (m, 1H).

Precursor Compound A



23

-continued



Precursor Compound B

5

10

15

## SYNTHESIS EXAMPLE 3

## Synthesis of Precursor Compound B

1,5-Dihydroxynaphthalene (40.0 g, 0.25 mol) was dissolved in 300 ml of dioxane, and ground sodium hydroxide (10.0 g, 0.25 mol) was added. The mixture was stirred for 30 min, and tetrabutylammonium hydrogen sulfate (0.46 g) was added. To this mixture was added methacryloyl chloride (26.1 g, 0.25 mol) in dioxane (120 ml). The reaction was stirred at room temperature for 3 hours and the precipitate was filtered off. The crude product was purified by column chromatography on silica gel using 15:85 ether:hexane mixture as an eluent to give 28.5 g of Precursor Compound B (shown above) as an off-white powder (50% yield). <sup>1</sup>H NMR (CD<sub>3</sub>OD) δ ppm: 2.16 (s, 3H), 5.86 (s, vinyl H, 1H), 6.25 (s, br, OH, 1H), 6.53 (s, vinyl H, 1H), 7.12–7.40 (m, 5H), 7.94 (d, d=8.4 Hz, 1H).

## SYNTHESIS EXAMPLE 4

## Synthesis of Precursor Polymers C and D

Precursor Compound B (10.0 g, 0.044 mol) and azobisisobutyronitrile (AIBN, 0.14 g) were dissolved in methanol (50 ml). The solution was purged with dry nitrogen and then heated to 57° C. overnight. The resulting polymer was precipitated into water twice. The resulting white powdery Precursor Polymer D (shown below) was dried under vacuum at 60° C. in the presence of phosphorus pentoxide overnight (9.2 g, 92%).

Precursor Polymer C (shown below) was prepared similarly from Precursor Compound A.



Precursor Polymer C

24

-continued



Precursor Polymer D

20

25

30

35

40

## SYNTHESIS EXAMPLE 5

## Synthesis of Polymers 6–8

Precursor Polymer C (3.0 g) was dissolved in absolute methanol (20 ml) and the solution was cooled to 0° C. HCl gas was bubbled through it for 30 min and tetrahydrothiophene (1.7 g) in methanol (10 ml) was added slowly to maintain the temperature below 0° C. HCl gas was bubbled through the solution for another hour. The resulting polymer was precipitated into water, filtered and dried to give 3.85 g off-white solid Polymer 6 (76% yield). <sup>1</sup>H NMR analysis indicates that about 20% of the repeating units containing cyclic sulfonium moiety. The resulting polymer was dissolved in methanol, and neutralized with sodium methoxide. The polymer was precipitated from water, filtered and dried.

Polymer 7 was prepared similarly from Precursor Polymer D, and Polymer 8 was similarly prepared from a commercially available phenol-formaldehyde novolak resin (Monomer-Polymer & Dajac Laboratories, Inc., Mw of 5000). About 20 mol % of the recurring units of each of these three polymers contained the heat-activatable aromatic cyclic sulfonium zwitterion groups.

The following examples illustrate the practice of the invention, and are not meant to limit it in any way.

## INVENTION EXAMPLES 1–8

These examples illustrate imaging members of the present invention that have imaging layers that include thermally sensitive polymers or small molecule compounds, are coated on a polyester support, and are imaged developed on press.

A thermally sensitive imaging formulation was prepared from the following components:

|                                         |        |
|-----------------------------------------|--------|
| Thermally sensitive compound 1–5, 10–12 | 0.33 g |
| IR dye 7                                | 0.03 g |
| Water                                   | 2.5 g  |
| Methanol                                | 6.2 g  |

Each formulation containing 4 weight % of solids was coated to provide 100 mg/ft<sup>2</sup> of dry coverage (1.08 g/m) on 0.10 mm poly(ethylene terephthalate) support. The resulting printing plates were dried in a convection oven at 82° C. for 3 minutes, clamped onto the rotating drum of a conventional platesetter having an array of laser diodes operating at a wavelength of 830 nm each focused to a spot diameter of 23 mm at dosages ranging from 457 to 1141 mJ/cm<sup>2</sup>. Each channel provided a maximum of 450 mWatts (mW) of

25

power incident upon the imaging layer surface. The blue imaging layer coatings showed strong bluer images in the exposed regions.

A sample of each of the laser-exposed plates was then mounted on the plate cylinder of a conventional full-page A. B. Dick 9870 lithographic duplicator press for actual press runs using Varn Universal Pink fountain solution. The fountain solution simultaneously removes non-exposed regions of the imaging layers (development). Using VanSon Diamond Black lithographic printing ink, each printing plate provided a few thousand sheets with fill density images. The press results (number of acceptable sheets) are shown in the following TABLE I.

TABLE I

| Example | Thermally Sensitive Compound | Press Results (Printed Sheets) |
|---------|------------------------------|--------------------------------|
| 1       | 1                            | 1,000                          |
| 2       | 2                            | 1,000                          |
| 3       | 3                            | 1,000                          |
| 4       | 4                            | 1,000                          |
| 5       | 5                            | 1,000                          |
| 6       | 10                           | 1,000                          |
| 7       | 11                           | 1,000                          |
| 8       | 12                           | 1,000                          |

## INVENTION EXAMPLES 9-12

These examples illustrate imaging members of the invention that comprise aluminum supports and are developed by tap water or a commercial fountain solution. Imaging layers were provided as described in Examples 1-8 on 0.14 mm grained anodized aluminum sheets. The resulting imaging members were imaged as described above and developed with tap water or a commercial fountain solution. Printing results on the same A. B. Dick press are summarized in the following TABLE II.

TABLE II

| Example | Thermally Sensitive Compound | Developer Solution                                           | Press Results (Printed Sheets) |
|---------|------------------------------|--------------------------------------------------------------|--------------------------------|
| 9       | 1                            | Varn Universal Pink fountain solution 28 ml/3.8 liters water | 1,000                          |
| 10      | 1                            | Tap water                                                    | 1,000                          |
| 11      | 12                           | Tap water                                                    | 1,000                          |
| 12      | 12                           | Varn Universal Pink fountain solution 28 ml/3.8 liters water | 1,000                          |

## INVENTION EXAMPLES 13-20

These examples illustrate imaging members of the present invention that include carbon black as the photothermal conversion material.

Several heat-sensitive imaging formulations were prepared and coated on 0.14 mm grained, anodized aluminum, and dried as described in Example 1-8, except that carbon black (Nippon Shokubai FX-GE-003) was used instead of IR Dye 7. Each resulting plate was imaged and tested on the printing press as described in Examples 1-8 and used to acceptably print at least 1000 sheets.

The invention has been described in detail with particular reference to preferred embodiments thereof, but it will be understood that variations and modifications can be effected within the spirit and scope of the invention.

26

I claim:

1. A heat-sensitive composition comprising:
  - a) a thermally sensitive compound comprising a heat-activatable aromatic cyclic sulfonium zwitterion group represented by the following Structure I:



wherein Ar is a substituted or unsubstituted aromatic group, X and Y are independently substituted or unsubstituted methylene groups, and n is 1 or 2, and

- b) a photothermal conversion material.

2. The composition of claim 1 wherein Ar is a phenyl or naphthyl group that is unsubstituted or substituted with one or more halo, alkyl, aryl, alkoxy, ester, amine, thioether, or thioester groups, X and Y are independently —CH<sub>2</sub>— or —CHR—, R is a halo, alkyl, aryl, alkoxy, ester, amine, thioether, or thioester group, and n is 1.

3. The composition of claim 2 wherein Ar can be substituted with one or more chloro, bromo, or alkyl groups having 1 to 4 carbon atoms, and X and Y are both —CH<sub>2</sub>—.

4. The composition of claim 1 wherein said heat-sensitive composition comprises one or more thermally sensitive compounds represented by one or more of the following Structures I-a through I-k:

I-a



I-b



I-c



27

-continued

I-d  
5I-e  
15

20

I-f  
25

35

I-g  
40

45

50

I-h  
55

60

65

28

-continued

I-i



I-j

I-k



1



2

wherein R is the same or different substituent on the aromatic rings, Z is a divalent linking group, m is 0 or an integer representing the number of available open ring positions on the aromatic rings, and q is 0 or 1.

5. The composition of claim 4 wherein said heat-sensitive composition comprises one or more of the following compounds 1 to 5:

**29**

-continued

**30**

-continued



6. The composition of claim 1 wherein said photothermal conversion material is a carbon black or an IR dye that is bis(dichlorobenzene-1,2-thiol)nickel(2:1)tetrabutyl ammonium chloride, tetrachlorophthalocyanine aluminum chloride, or one of the following compounds:

IR Dye 1

IR Dye 2 is the same as IR Dye 1 but with  $C_3F_7CO_2^-$  as the anion.

IR Dye 3



IR Dye 4



31

32

-continued

IR Dye 5

IR Dye 6



IR Dye 7



IR Dye 8



IR Dye 9



IR Dye 10



-continued



IR Dye 11



IR Dye 12



IR Dye 13



IR Dye 14

7. The composition of claim 1 further comprising water, methanol, ethanol, 1-methoxy-2-propanol, or a mixture of two or more of these.

8. The composition of claim 1 wherein said thermally sensitive compound is present at from about 1 to about 90% solids, and said photothermal conversion material is present at from about 5 to about 35% solids.

9. A method of imaging comprising the steps of:

- A) spray coating the heat-sensitive composition of claim 1 onto a support to provide an imaging member, and
- B) imagewise exposing said imaging member with thermal energy to provide exposed and unexposed areas in the imaging layer of said imaging member, whereby said exposed areas are rendered more hydrophobic than said unexposed areas.

10. The method of claim 9 wherein said support is an on-press printing cylinder or sleeve.

11. A thermally sensitive imaging member comprising a support having disposed thereon, the same or different layer, a) a thermally sensitive compound comprising a heat-activatable aromatic cyclic sulfonium zwitterion group represented by the following Structure I:



35

wherein Ar is a substituted or unsubstituted aromatic group, X and Y are independently substituted or unsubstituted methylene groups, and n is 1 or 2, and

b) a photothermal conversion material.

12. The imaging member of claim 11 comprising a polyester or aluminum support.

13. The imaging member of claim 11 wherein said thermally sensitive compound is present in said imaging layer in an amount of at least 0.1 g/m<sup>2</sup>, and said photothermal conversion material is present in said imaging layer in an amount sufficient to provide a transmission optical density of at least 0.1 at 830 nm.

14. The imaging member of claim 11 wherein said support is an on-press printing cylinder.

15. A method of imaging comprising the steps of:

A) providing the imaging member of claim 11, and

B) imagewise exposing said imaging member with thermal energy to provide exposed and unexposed areas in the imaging layer of said imaging member, whereby said exposed areas are rendered more hydrophobic than said unexposed areas.

16. The method of claim 15 wherein said imagewise exposing is carried out using an IR radiation emitting laser, and said imaging member is a lithographic printing plate having an aluminum support or an on-press imaging cylinder having a cylindrical support.

17. The method of claim 15 wherein said imagewise exposing is accomplished using a thermal head.

18. A method of printing comprising the steps of:

A) providing the imaging member of claim 11,

B) imagewise exposing said imaging member with thermal energy to provide exposed and unexposed areas in the imaging layer of said imaging member, whereby said exposed areas are rendered more hydrophobic than said unexposed areas, and

C) with or without wet processing, contacting said imagewise exposed imaging member with a lithographic printing ink, and imagewise transferring said printing ink from said imaging member to a receiving material.

19. A heat-sensitive composition comprising:

a) a thermally sensitive polymer represented by the following Structure II:



wherein A represents a polymeric backbone, Ar' represents a divalent aromatic group, R represents the same or different substituent on said aromatic group, m is 0 or an integer representing available open ring positions on Ar', n is 1 or 2, q is 0 or 1, X and Y are independently substituted or unsubstituted methylene groups, and Z is a divalent linking group, and

b) a photothermal conversion material.

20. The composition of claim 19 wherein A is a vinyl polymeric backbone, Ar' is a phenylene or naphthylene group, R is a halo, alkyl, aryl, alkoxy, ester, amine, thioether, or thioester group, m is 0 or an integer of from 1 to 3, X and Y are independently —CH<sub>2</sub>— or —CHR—, and n is 1.

36

21. The composition of claim 20 wherein R is a chloro, bromo, or an alkyl having 1 to 4 carbon atoms, m is an integer of from 1 to 3, X and Y are both —CH<sub>2</sub>—.

22. The composition of claim 19 wherein Z is —(Z)<sub>p</sub>Z'<sub>t</sub>— wherein Z' is an oxy, thio, carboxyloxy, oxycarbonyl, carbonyl, carbonyloxycarbonyl, —SO—, —SO<sub>2</sub>, —NHCONH—, or carbonamido group, Z" is an alkylene, arylene, arylenealkylene, or alkylenearylene group, p and t are independently 0 or 1.

23. The composition of claim 22 wherein Z is —COO— or —COOZ" wherein Z" is an alkylene group of 1 or 2 carbon atoms, a phenylene group, or a naphthylene group, and p and q are each 1.

24. The composition of claim 23 wherein Z is —COO—.

25. A thermally sensitive imaging member comprising a support having disposed thereon one or more layers comprising:

a) a thermally sensitive polymer represented by the following Structure II:



35 wherein A represents a polymeric backbone, Ar' represents a divalent aromatic group, R represents the same or different substituent on said aromatic group, m is 0 or an integer representing available open ring positions on Ar', n is 1 or 2, q is 0 or 1, X and Y are independently substituted or unsubstituted methylene groups, and Z is a divalent linking group, and

b) a photothermal conversion material.

26. A heat-sensitive composition comprising:

a) a thermally sensitive compound represented by the following Structure III:



55 wherein X' represents polymer recurring units, SULFO represents heat-activatable aromatic cyclic sulfonium zwitterion groups, and Y' represents recurring units derived from any additional ethylenically unsaturated polymerizable monomers, x is from about 10 to 100 mol %, and y is from 0 to about 90 mol %, and

b) a photothermal conversion material.

27. The heat-sensitive composition of claim 26 wherein said compound of Structure III is Compound 6, 7, or 8:

37



**28.** A thermally sensitive imaging member comprising a support having disposed thereon one or more layers comprising:

a) a thermally sensitive compound represented by the following Structure III:



wherein X' represents polymer recurring units, SULFO represents heat-activatable aromatic cyclic sulfonium zwitterion groups, and Y' represents recurring units derived from

38

any additional ethylenically unsaturated polymerizable monomers, x is from about 10 to 100 mol %, and y is from 0 to about 90 mol, and

b) a photothermal conversion material.

29. A thermally sensitive imaging member comprising a support having disposed thereon one or more layers comprising:

a) a mixture of two or more of the thermally sensitive compounds represented by any of the following Structures I, II, and III:



wherein Ar is a substituted or unsubstituted aromatic group, X and Y are independently substituted or unsubstituted methylene groups, and n is 1 or 2,



wherein A represents a polymeric backbone, Ar' represents a divalent aromatic group, R represents the same or different substituent on said aromatic group, m is 0 or an integer representing available open ring positions on Ar', q is 0 or 1, and Z is a divalent linking group, and



wherein X' represents polymer recurring units, SULFO represents heat-activatable aromatic cyclic sulfonium zwitterion groups, and Y' represents recurring units derived from any additional ethylenically unsaturated polymerizable monomers, x is from about 10 to 100 mol %, and y is from 0 to about 90 mol, and

b) a photothermal conversion material.

\* \* \* \*